

# UNITED STATES PATENT OFFICE.

BENJAMIN H. DOSENBACK, OF BUTTE, MONTANA.

## ORE-CONCENTRATION PROCESS.

1,257,329.

specification of Letters Patent. Patented Feb. 26, 1918.

No Drawing.

Application filed November 16, 1917. Serial No. 202,267.

To all whom it may concern:

Be it known that I, BENJAMIN H. DOSENBACK, a citizen of the United States, residing at Butte, in the county of Silver Bow 5 and State of Montana, have invented certain new and useful Improvements in Ore-Concentration Processes, of which the following is a specification.

My invention is an improved flotation process. In the flotation processes as previously practised certain reagents generally termed modifying agents or oils, although many of such substances are not oils, properly speaking, are added to a freely flowing 15 pulp whereupon the introduction of air or some other gas into the pulp gives rise to the formation of bubbles which collect the desired material, generally metalliferous sulfids, and reject the gangue. The modifying 20 agents used for this purpose comprise a great variety of oils, animal, vegetable and mineral oils, coal and wood tar and derivatives thereof, various alcohols, hydroxyl compounds and other substances, all of 25 which are referred to herein as oils or modifying agents for want of a better generic term. Air, of course, is the most available gas and the one generally used, but in referring to air I include other gases which may 30 be substituted with similar results.

A procedure heretofore widely used in the application of the principles above referred to consists in adding the modifying agent to the ore pulp and then subjecting 35 the mixture to violent mechanical agitation with the result of beating air into the pulp, after which the mixture is brought to a state of substantial quiescence, whereupon the air rises in the form of bubbles and floats the 40 concentrate as a froth. Such a procedure is described in numerous United States patents and in various publications. Another method of procedure consists in the introduction of air through a porous medium 45 such as canvas, unglazed earthenware or other porous medium, which has the effect of minutely subdividing the air and introducing it to the pulp in the form of very small bubbles, which rising through the 50 pulp collect the desired solid constituents thereof and form a bubble column above the normal pulp level, that is, the level assumed by the pulp before the introduction of air. By permitting the upper part 55 of the bubble column to overflow efficient concentration is obtained, the overflowing

bubbles carrying with them the selected mineral. Such a procedure is also well known in the art. It has heretofore been discovered that it is not necessary to mix the modifying agent with the water and solids constituting the ore pulp, but that it is sufficient to introduce the modifying agent in the form of a vapor or gas with the air. I have discovered furthermore, that in such a mode of procedure it is unnecessary that the modifying agent mixed with the air be in the gaseous or vaporized form, but that efficient results are obtained if the modifying agent in the liquid form is minutely subdivided, so minutely subdivided as to be carried with the stream of air in the form colloquially referred to as a "fog." The modifying agent may be reduced to the condition stated by means of an ordinary atomizing device wherein a stream of air or other medium is caused to impinge upon the oil at high velocity. This atomizing operation is carried out completely before the air carrying the oil is introduced into the pulp, that is, after the air has been impregnated with finely divided modifying agent it is conducted to the concentration vessel where it is introduced into the ore pulp through some porous medium. In my improved process the modifying agent is not injected into the pulp by means of an atomizer or injector, but a mixture of air with a modifying agent so finely divided as to remain suspended in the air is prepared in advance and a mixture of air and modifying agent so prepared is then conducted to and introduced into the ore pulp through a porous medium.

The form of the mixture of modifying agent with air which I utilize in my process is best described as a fog, this being the term used in the gas making art to describe an analogous mixture consisting of the gases resulting from distillation in admixture with certain tar products which condense to the form of a fog upon the collecting of the gas after it leaves the retorts. In the gas manufacturing art it is necessary to remove this fog from the gases before delivery thereof to the service mains, but in practising my invention I utilize a fog of this character and can prepare the necessary medium for flotation use by distilling gases from coal, asphaltic matter, gilsonite and other substances, and conducting the gases formed to the flotation apparatus without

removing the fog therefrom, or without removing all of it. My invention includes the use of such fogs whether created by atomizing a liquid as hereinbefore referred to, or 5 whether their existence grows out of a process of distillation of such substance as above referred to.

In the foregoing references to the use of atomizers for producing the fog referred to 10 I do not intend to convey the idea that my invention consists in the use of a stream of what is popularly known as "atomized" liquid. Such a stream of atomized liquid carries liquid globules which, while comparatively small, are of such size that they 15 immediately settle out of and separate from the stream of air, in fact remain in suspension only so long as the air is in motion. A familiar example of such "atomized" liquid 20 is presented by an ordinary scent spray the liquid particles in which settle and collect into a mass immediately the blast of air is arrested, as by the hand placed before the nozzle of the scent spray apparatus. The 25 medium used in my process is not a spray of this kind containing liquid particles so large as to settle and collect into a mass when the air stream comes to rest, but is a body or stream of air carrying liquid or 30 solid particles so minute that they remain in suspension even when the air is quiescent. A spray, or "atomized" liquid, consists of liquid particles analogous to rain drops, which settle and fall; the fog which I uti-

lize is analogous to the atmospheric condition in foggy weather, the particles of liquid 35 being so minute that they remain in suspension even in quiet air. I have found that an atomizer in which a stream of air impinges upon liquid particles, while producing under some conditions a considerable amount of ordinary spray which immediately settles and gathers in masses, also reduces part of the liquid to the condition of the true fog which I utilize in my improved 40 process. When using an atomizer in my improved process if any of the comparatively large globules which settle when the air comes to rest are produced these large globules are permitted to settle and only the part of the 45 liquid which is reduced to the condition of a true fog is utilized.

What I claim is:

An ore concentration process comprising the operations of forming a mixture of air 55 with a modifying agent in the form of a fog, introducing said mixture through a fine texture porous medium into an ore pulp, forming bubbles to which certain mineral particles in the ore adhere as said bubbles rise 60 through the pulp, causing said mineral bearing bubbles to form a column of bubbles above the pulp and separating the mineral carried by the bubbles from the remainder of the ore.

In testimony whereof, I have subscribed my name.

BENJAMIN H. DOSENBACH.